

## UNITED STATES PATENT OFFICE

2,368,670

## LUBRICATING COMPOSITION

Bert H. Lincoln and Gordon D. Byrkit, Ponca City, Okla., assignors, by mesne assignments, to The Lubri-Zol Development Corporation, Cleveland, Ohio, a corporation of Delaware

No Drawing. Application October 6, 1939,  
Serial No. 298,337

1 Claim. (Cl. 252—48)

This invention relates to lubricating oils and more particularly to improved lubricating oils of high film strength, high resistance to oxidation, and markedly reduced formation of corrosive products during use.

Present-day mechanical devices require lubricating oils of high film strength, of high oiliness characteristics, and of low tendency to oxidize during use. It has been found that the present-day hydrocarbon lubricants of the very highest quality are deficient in these very important characteristics. These three properties are of vital importance under conditions of thin film lubrication where the lubricant has been squeezed from between the friction surfaces because of high pressure, slow speeds, and other causes. In modern engines, large surfaces of oil are exposed to the action of atmospheric oxygen, promoting rapid oxidation. It is readily seen that the viscosity or the body of the lubricant plays no part in thin film lubrication and that the remaining film of oil must have a very high film strength and be of high oiliness value to prevent rupture of the film of the lubricant, which would cause seizure. The oil film must tend to keep the coefficient of friction as low as possible. The oil must resist oxidation when these thin film are heated in the presence of atmospheric oxygen as they are in use.

Mechanical devices are being designed for higher pressure operation, and the film strength of the best quality straight hydrocarbon lubricant has been found to be too low for satisfactory service. It will be obvious that an invention which provides a means of improving the film strength of these lubricants is of great importance to the art of lubricant manufacture and to the designer and fabricator of mechanical devices.

Substantially all machines operate in part or at times totally under conditions of boundary or thin film lubrication, under which conditions the oiliness or unctuousness of the lubricant is the first and primary requisite of efficient operation. Those skilled in the art of lubricant manufacture or machine manufacture will readily appreciate the value of an invention that will improve the oiliness of these otherwise high-quality lubricants. Furthermore, sludge and acid are especially deleterious under conditions of thin film lubrication. The sludge is not a lubricant in any sense of the word, and the soluble acid is particularly corrosive to bearing metals such as cadmium-silver, copper-lead, and the like.

In starting idle mechanical equipment which is lubricated from a sump by pumping or circulating the lubricant, there is always a short period of

time in which the rubbing surfaces must operate under conditions of dry friction if ordinary hydrocarbon lubricants are used. With dry friction, the wear on friction surfaces is extreme; and during cold weather when the lubricant is sluggish or during periods when the lubricating system is not functioning properly for one reason or another, rubbing surfaces may not only suffer considerable wear but may be damaged to the point where they must be replaced. The product of our invention has a very important property of reacting with the metal surfaces, penetrating or absorbing on the metal surfaces, and leaving a film of lubricant with high oiliness character, which remains on the metal surface irrespective of the length of time the machine has been idle.

This high oiliness film gives very even and smooth operation, which may be easily discerned by the experienced operator or lubricating engineer.

When the hydrocarbon lubricants are diluted with unburned fuel or with other light hydrocarbons, the small degree of oiliness of the original hydrocarbon lubricant is greatly decreased. We have found that the addition of the products of our invention to hydrocarbon lubricants more than compensates for the loss in oiliness and load-carrying ability from dilution.

It is well known that, in order to obtain lubricants which are preeminently satisfactory from the standpoint of oxidation in use, it is necessary to refine the oil thoroughly and then to add an inhibitor of oxidation. The thorough refining may consist of more and heavier acid treatments or solvent treating so as to remove a considerable part of the oil and leave only the most stable portion. Such drastic refining is necessary in order to obtain stability with respect to sludge formation, but the oil is then subject to easy oxidation to form soluble acids and other corrosive materials. This can be prevented by the addition to the refined oil of small amounts of materials which either prevent the formation of these corrosive products or by some action render them inert. Furthermore, such well-refined oils are susceptible to the formation during use of lacquer-like materials which tend to stick rings. This results in blow-by and hence loss of power, failure of lubrication, scratching, scoring, overheating, and eventual replacement of parts. It is practically impossible to refine a lubricant in such a manner as to avoid all three of these difficulties, namely, soluble corrosive products, sludge, and lacquer. It is considerably more ad-

vantageous to add the materials of our invention and avoid these difficulties by this method.

Certain compounds are adsorbed or absorbed by metals thus forming tenacious films at the surface of metals; these films are able to stand high pressures. X-ray diffraction methods have shown that compounds containing highly polar molecules, that is, molecules of unsymmetrical electrical character containing an atom or group of atoms exhibiting a secondary or residual valence, tend to produce regimentation of the molecules of hydrocarbon oil when added thereto. A metal immersed in a strongly polar compound will show a film of the compound in which there is a regimentation of molecules oriented with respect to the surface of the metal by which they are adsorbed or absorbed.

Many of our additive materials are effective when added to poorly refined or even wholly unrefined lubricants. The addends may thus be substituted in whole or in part for the usual refining processes.

In the prior art of applying these principles to the manufacture of lubricants, many diverse types of materials have been suggested to be added to obtain improvement in various characteristics. It has been found that the addition of various compounds frequently improves film strength, oxidation resistance, noncorrosiveness, and other characteristics.

One object of our invention is to provide improved inhibitors of oxidation and corrosion for addition to lubricants.

Another object of our invention is to provide film strength improving addition agents suitable for use in lubricants and especially in crankcase lubricants.

Other and further objects of our invention will appear in the course of the following description.

To the accomplishment of the foregoing and related ends, said invention, then, consists of the means hereinafter fully described and particularly pointed out in the claims.

In general, our invention contemplates an oil of lubricating viscosity having added thereto a small amount of an organic thiocarbonate of the general formula



in which C represents carbon, X represents either oxygen or sulfur (at least one of the X's must be sulfur) and R and R' are organic radicals one or both of which contain carbon, hydrogen, and at least one other element besides halogen. Halogen may be present in the R's but in that case another characterizing element must also be present. The elements which we refer to here as "characterizing elements" include oxygen, sulfur, selenium, tellurium, nitrogen, phosphorus, arsenic, and metallic elements, such as, tin, antimony, bismuth, and the like. The R's may be aliphatic, carbocyclic, or heterocyclic in character. It will be apparent that by thiocarbonate in the appended claims we mean to include mono- and trithiocarbonates as well as the di-thiocarbonates (xanthates).

The introduction of this characterizing element into our thiocarbonates permits of an extraordinary flexibility in the design of the addend for a particular use. Thus it permits the introduction of additional sulfur if the sulfur in the thiocarbonate is insufficient in amount or the introduction of other forms of sulfur if the thio-

carbonate sulfur is too stable or too unstable. The additional inhibiting action of phosphorus, nitrogen, or organo-metallic groups may be added to the molecule to produce an extremely effective inhibitor of oxidation and/or corrosion. Furthermore the newly introduced elements have a considerable effect on the activity of the thiocarbonate sulfur and it may be activated or depressed by the use of suitable groups in the R's of our thiocarbonates. Chlorine may in turn have an activating effect on the characterizing element or elements.

The substituted thiocarbonates of our invention show an unexpected improvement over the corresponding unsubstituted thiocarbonates and even over mixtures of the unsubstituted thiocarbonates with other compounds having the same substituting groups. Thus a xanthate containing a triphenyltin group in the organic radical shows a greater effect as an antioxidant than the triphenyltin group in, say, tetraphenyltin plus the same xanthate without the triphenyltin group. Similar unexpected results are obtained on the introduction of oxygen as an oiliness factor, halogen, nitrogen, phosphorus, sulfur metal and the like as film strength or inhibiting factors.

The particular thiocarbonates of this invention have a dual action in a lubricant. One action involves increased load-carrying ability and/or oiliness, while another action is directed to the stability of the lubricant. For load-carrying capacity, quantities ranging from 0.1 per cent to about 10 per cent may be added. As an anti-corrosive agent and/or an anti-sludging agent, much smaller amounts may be required ranging from approximately 0.001 to 1.0 per cent. The action of our thiocarbonates is specific but difficult to understand. These compounds may be added to any type of hydrocarbon lubricants but show an unusual value in highly refined and solvent treated lubricants. By oil having lubricating viscosity in the appended claims, we mean to include the so called mineral oils and various hydrogenated, polymerized and otherwise synthetically treated oils such as volatilized oils, aluminum chloride treated oils, and the like. Furthermore the lubricating oil may consist in whole or in part of shale oil, animal or vegetable oils such as castor oil, lard oil, corn oil, cottonseed oil, and the like.

In practice, it is better to employ compounds whose boiling point is above 250° F. in order that the addition compound will not be evaporated or distilled in use. The selection of a particular compound or compounds to be used as an addition agent to the hydrocarbon or other oil is to be made considering the physical and chemical properties of the various compounds and the use to which the blend is put. Thus, if water is likely to be present during use, a salt or combination of salts is selected which is not affected by water. If a particular added compound proves too volatile for its application, a higher boiling material should be used and the more volatile compound used for blending in an oil intended for duty at lower temperatures. In general, for automotive crankcase lubricants, we prefer to use compounds having vapor pressures of less than atmospheric at 250° F.

70 The following compounds may be used in accordance with our invention. All and each of these are to be considered as examples of our invention when blended in minor proportion in an oil of lubricating viscosity.

75 One or both of the organic radicals in our

mono-, di-, or trithiocarbonates may be of various types as shown in the following classification. Each of the following organic, or organo-metallic radicals may be combined with mono-, di- and trithiocarbonate radicals as further examples of our invention.

## I.—Aliphatic types

## A. Containing oxygen

## a. Alcohols

1. Hydroxyethyl ethylxanthate
2. Reaction product of potassium laurylxanthate and glycerol monochlorohydrin or glycerol dichlorohydrin.
3. Reaction product of potassium ethoxyethylxanthate with chlorinated, hydroxylated paraffin wax which has been chlorinated to 20 per cent chlorine and had half the chlorine removed by treatment with aqueous caustic under pressure to form the hydroxy compound.

## b. Ethers

4. Butoxyethyl butoxyethylxanthate
5. Reaction product of potassium amyltrithiocarbonate with paraffin wax chlorinated to 23 per cent chlorine and treated with sodium butylate to remove about one-third of the chlorine to make the butyl ether
6. Reaction product of potassium amylxanthate with beta, beta prime-dichloroethyl ether.

## 7. Methyl ethoxyamylxanthate

8. Reaction product of potassium amylxanthate with chloroacetone
9. Reaction product of potassium amylxanthate with symmetrical dichloroacetone so as to form di(amyloxanthylmethyl) ketone.
10. Reaction product of potassium amylxanthate with symmetrical dichloroacetone so as to form amylxanthylmethyl chloromethyl ketone
11. Unsaponifiable oxidation products of paraffin wax chlorinated and part or all of the chlorine removed by condensation with sodium ethylxanthate

## d. Aldehydes

12. Alpha-butyloxanthylbutyraldehyde
13. Alpha-ethoxyethylxanthylbenzaldehyde

## e. Acids and salts

14. Alpha-amylxanthylstearic acid
15. Calcium amylxanthylchlorostearate
- 15a. Tin amylxanthylchlorostearate
16. Ethoxyethylxanthylphenylstearic acid
17. Aluminum ethoxyethylxanthylphenylstearate

## f. Esters

18. n-Butyl ethylxanthylacetate  
A mixture of 65 parts of finely powdered potassium ethylxanthate, 65 parts of n-butyl chloroacetate, and 200 parts of acetone was agitated and heated for five hours. The acetone solution was drawn off, concentrated, and the residual oil distilled at 128-135 at one mm. pressure.

19. Methyl ethylxanthylchlorostearate  
A mixture of 48 parts of finely powdered potassium ethylxanthate, 102.5 parts of methyl dichlorostearate, and 100 parts of acetone was similarly refluxed and separated. The residual oil contained 4.05 per cent sulfur. A one per cent blend of this material in a S. A. E. 30 mineral oil showed a Timken film strength of 28 pounds on the arm. The mineral oil alone had a Timken film strength of only 9 pounds on the arm.

## g. Amides

20. Amylxanthylsuccindiamide
21. Laurylxanthylauramide

## B. Containing sulfur

## a. Mercaptans

22. Mercaptoamyl butoxyethoxyethylxanthate

## b. Sulfides and polysulfides

24. Reaction product of sodium laurylxanthate with beta, beta prime-dichloroethyl sulfide
25. Reaction product of sodium amyltrithiocarbonate with dichloroamyl trisulfide

## c. Thioacids and derivatives

26. Reaction product of sodium amylmonothiocarbonate with methyl alpha-chlorothiostearate
27. Reaction product of lithium isobutylxanthate with alphabromothiovaleramide

## d. Sulfones and sulfoxides

28. Reaction product of sodium ethoxyethylxanthate with omega-chloroamylsulfone
29. Reaction product of sodium hexylxanthate with omega-chloroamylsulfoxide

60

65

70

75

## e. Sulfurized aliphatic compounds

30. Reaction product of potassium hexylxanthate with sulfur and chlorine bearing methyl oleate
31. Reaction product of potassium ethylxanthate with sulfur chloride treated methyl linoleate
32. Reaction product of potassium benzylxanthate with sulfur chloride treated methyl esters of soy bean or corn oil acids

## C. Containing nitrogen

## a. Amines

33. Beta-aminoethyl ethylxanthate
34. Reaction product of potassium octadecylxanthate with 3-amino-2-chloropentane

35. Reaction product of potassium amylxanthate with 3-dimethylamino-2-chloropentane

## b. Nitro compounds

36. Omega-nitroamyl amylxanthate
37. Reaction product of potassium butylxanthate with nitro-chloro-paraffin wax

## c. Cyanides, isocyanides, thiocyanides, cyanates

38. Thiocyanato-ethyl laurylxanthate
39. Reaction product of sodium ethoxyethylxanthate with chloroacetonitrile

40. Reaction product of sodium propylxanthate with omega-chloroamyl isocyanide
41. Reaction product of sodium amylxanthate with omega-chloroamyl cyanate

## D. Containing phosphorus

42. Tri(ethoxyethylxanthyl)phosphate
43. Tri(ethoxyethylxanthyl)phosphite
44. Tri(ethoxyethylxanthyl)thiophosphate
45. Methyl butoxyethylxanthyl phosphino-stearate
46. Diethylphosphinoethyl amylxanthate

## E. Containing metals

## a. Group IV

47. Triethylstannylamyl amylxanthate
48. Triethylplumbylethyl amyltrithiocarbonate
49. Triamylstannylethyl ethoxyethylxanthate

## b. Group V

50. Diethylarsenylamyl ethylxanthate
51. Diethylantimonyl amyl ethylmonothiocarbonate
52. Diethylbismuthylamyl ethylxanthate

## c. Group VI

53. Amylseleniummethyl ethoxyethylxanthate
54. Amyltelluriummethyl butylxanthate

## II.—Carbocyclic types

## A. Containing oxygen

## a. Phenols

55. Hydroxyphenyl ethylxanthate
56. Omega-hydroxyphenylamyl amylxanthate

57. Reaction product of potassium amylxanthate with chlororesorcinol
58. Reaction product of potassium amylxanthate with halogenated paraffin wax substituted phenol

## b. Alcohols

59. Reaction product of sodium butoxyethylxanthate with o-chlorobenzyl alcohol
60. Reaction product of sodium butylxanthate with hydroxylated, halogenated phenylated wax

## c. Ethers

61. Anisyl laurylxanthate
62. Omega-phenoxyamyl amylxanthate
63. Phenoxyphenyl laurylxanthate
64. Reaction product of potassium benzylxanthate with chlororesorcinol dimethyl ether

## d. Ketones

65. Reaction product of sodium ethylxanthate with chlorobenzophenone
66. Omega-amylxanthylacetophenone
67. Reaction product of potassium isobutylxanthate with chlorostearoylterinalin

## e. Aldehydes

68. Reaction product of sodium benzylxanthate with o-chlorobenzaldehyde
69. Reaction product of sodium ethoxyethylxanthate with omega-chlorotolu-aldehyde

## f. Acids and salts

70. Reaction product of potassium amylxanthate with cinnamic acid dichloride
71. Reaction product of sodium ethylxanthate with chlorine-bearing dinaphthylstearic acid
72. Calcium salt of the reaction product of sodium laurylxanthate with o-chlorobenzoylbenzoic acid

## g. Esters

73. Reaction product of potassium amylxanthate and chlorinated phenyl benzoate
74. Phenyl ethoxyethylxanthyl phenylstearate

75. Chlorinated wax condensed (Friedel-Crafts) with phenyl benzoate and sodium amylixanthate
- h. Amides
76. Potassium butoxyethylxanthate condensed with chloro-stearanilide
77. Chloro-amylixanthylsteartoluidide
- B. Containing sulfur
- a. Mercaptans and thiophenols
78. Mercapto-dodecahydro-diphenyl ethylxanthate
79. Reaction product of potassium butyl-monothiocarbonate and o-chlorophenyl ethylmercaptan
- b. Sulfides and polysulfides
80. Reaction product of chlorobenzyldisulfide and potassium hexyltrithiocarbonate
81. Reaction product of sodium amylixanthio-carbonate and chlorophenylethyl disulfide
82. Reaction product of sodium amyl-monothiocarbonate with chlorodiphenyltrisulfide
83. Reaction product of potassium amylixanthate with chlorodiphenylsulfide
- c. Thioacids and derivatives
84. Reaction product of sodium laurylxanthate with omega-chlorothiobutolide acid
85. Reaction product of sodium benzylxanthate with alphabromothiobutyramide
- d. Sulfones and sulfoxides
86. Reaction product of potassium octadecylxanthate with chlorodiphenylsulfone
87. Reaction product of potassium ethyltrithiocarbonate with chlorodibenzylsulfone
88. Reaction product of sodium ethylmonothiocarbonate with chlorodibenzylsulfone
- C. Containing nitrogen
- a. Amines
89. Reaction product of lithium butylxanthate with chlorodiphenylamine
90. Reaction product of sodium benzylxanthate with o-chlorodimethylaniline
- b. Nitro compounds
91. Nitrocresyl thiocarbonate
92. Amyl nitrobenzylxanthate
- c. Azo compounds
93. Reaction product of potassium amylixanthate with the product of coupling diazotized p-chloroaniline with alpha-naphthol
- D. Containing phosphorus
94. Reaction product of sodium ethoxyethyl trithiocarbonate with chlorophosphazobenzene
95. Reaction product of sodium butoxyethoxyethylxanthate with p-chlorophosphinobenzene
- E. Containing metals
96. Reaction product of triphenyl-omega-chloroamyltin with sodium amylixanthio-carbonate
97. Triethylstannylylphenyl benzylxanthate
98. Triethylplumbylphenyl amylixanthate
99. Ethylmercuriphenyl amylixanthate
- III—Heterocyclic types
- A. Containing oxygen
100. Reaction product of potassium butylxanthate with chlorodioxane
101. Reaction product of potassium ethylxanthate with chlorodiphenylene oxide
102. Reaction product of chlorohydroxy-thiophene with sodium butoxyethylxanthate
- B. Containing sulfur
103. Reaction product of potassium ethoxyethylxanthate with chlorothianthrene
- C. Containing nitrogen
104. Reaction product of potassium amylixanthate with alpha-chloropyridine

Any of these compounds or other members of the classes represented may be used within the scope of our invention.

The thiocarbonates have varying degrees of solubility in hydrocarbon and other oils. In some cases it is necessary to use a solvent for the compound or to form colloidal suspensions of the compound in oil. While some of these compounds have only limited solubility in hydrocarbon oils, it is to be remembered that because of their great efficiency extremely small amounts are often effective. Thus we may use as little as 0.001 per cent of some of these compounds, and it will be seen that a fairly insoluble material may dissolve to a sufficient extent to be satisfactory for our purpose. In general, more than 0.001 per cent of

our addition agents are used, and we may add one, two, or even five per cent or more.

Furthermore, it is well known that different types of oils have different capabilities of dissolving a given material. For some purposes therefore, we prefer paraffinic, for other purposes, asphaltic, and for still other purposes, naphthenic or mixed base lubricants. Another method of obtaining a satisfactory mixture of addition agent 10 with the hydrocarbon oil is the use of a mutual solvent to bring the addend into solution. Alternatively, peptizing agents may be added to maintain the thiocarbonates in permanent suspension.

Many of the more difficultly soluble materials are rendered more soluble by the introduction of alkyl groups, particularly those containing four or more carbon atoms. The isoamyl, octyl, lauryl, and octadecyl radicals and radicals from paraffin wax greatly increase the solubility of organic compounds in oil. One or more of such groups may be introduced as required.

It is sometimes advantageous to combine more than one of these compounds in a blend to obtain particular properties. We accomplish this by mixing two or more of these compounds together and blending the mixture with the hydrocarbon oil or by blending one in the hydrocarbon oil, blending the second into this mixture, and so on until the composition is complete.

The various thiocarbonates usually improve both the film strength and oxidation characteristics of the hydrocarbon oil. For example, the sludging tendencies may be decreased by as little as 0.001 per cent of our thiocarbonates. The oxidation characteristics of lubricants are very important, and these are markedly improved by our compounds. The ability to reduce friction is another feature contributed to lubricants by some of our compounds.

It may be desirable to include in one and the same blend, in addition to the addends here described, other addends for specific purposes. Thus, we may add a pour point depressor such as a naphthalenechlor wax condensation product, a viscosity index improver such as certain resins or polymerized hydrocarbons, and sulfur or phosphorus containing inhibitors, such as alkyl and aryl phosphite esters and alkyl and aryl phosphate esters in addition to our thiocarbonates. Furthermore, various metallic compounds may be added to the blend without interfering with the action of our ingredients. Indeed, in some cases it is advantageous to combine with our compounds in a hydrocarbon oil blend such materials as calcium dichlorstearate, sodium stearate, sodium oleate, sodium chloroate, tin oleate, sodium naphthenates, tin naphthenate, chromium oleate, aluminum stearate, and other metallic soaps or inorganic-organic salts.

Our invention also contemplates the use in lubricating compositions comprising a major proportion of lubricating oil of minor amounts of the previously identified sulphur compounds with a separate organic halogen compound. The halogen compounds which may thus be employed may be classified as follows:

*Cyclic compounds, such as halogenated*

- 70 I—Benzenes and related compounds such as:
- (1) Halogenated benzene, e. g.  
    (a) Chlorinated benzene, e. g.  
        The dichlorbenzenes, notably the ortho compound  
(b) Brominated benzene, e. g.  
        Ortho-dibrom benzene  
(c) Fluorinated benzene

- (2) Halogenated derivatives of benzene such as:
- (a) Halogenated homologs of benzene, e. g.:
    - Mono-chlor toluene
    - Mono-chlor xylene
    - Mono-chlor cymene
    - Ethyl mono-chlor benzenes
    - Propyl mono-chlor benzenes
    - Di-ethyl dichlor benzenes
    - Propyl dichlor benzenes
    - Di-ethyl tetrachlor benzenes
  - (b) Halogenated amino derivatives of benzene, e. g.:
    - Chlorinated aniline
    - Mono-chlor aniline (preferably the ortho-compound)
    - Mono-chlor di-methyl aniline
    - Chlorinated toluidines
    - Chlorinated xylylides
    - Chlorinated diphenylamine
  - (c) Halogenated hydrobenzenes, e. g.:
    - Hydrogenated dichlor-benzenes
    - Dichlorohexahydrobenzene (Dichlor cyclohexane)
- II—Polyphenyls, and related compounds, including diphenyl, diphenyl benzenes, etc., such as
- (1) Halogenated diphenyl, e. g.:
    - (a) Chlorinated diphenyl, e. g.:
      - Mono-chlor diphenyls
      - Di-chlor diphenyls
      - Tri-chlor diphenyls
    - (b) Brominated diphenyl, e. g.:
      - The mono-brom diphenyls
    - (c) Fluorinated diphenyl
  - (2) Halogenated derivatives of diphenyl, such as:
    - (a) Halogenated homologs of diphenyl, e. g.:
      - Chlorinated phenyl-toluenes
      - Ethylenated, or propylated, chlorinated diphenyl, e. g. di-ethyl tetrachlor diphenyl
    - (b) Halogenated amino derivatives of diphenyl, e. g.:
      - Chlorinated phenyl-anilines
      - Chlorinated phenyl-toluidines
      - Chlorinated diphenyl amines (xenyl amines)
    - (c) Halogenated hydrodiphenyls, e. g.:
      - Chlorinated phenyl hexahydrobenzene
      - Chlorinated dodecahydronaphthalene
- III—Naphthalene and related compounds, such as
- (1) Halogenated naphthalene:
    - (a) Chlorinated naphthalene, e. g. -mono-chlor naphthalene
    - (b) Brominated naphthalenes, e. g. -mono-brom naphthalene
    - (c) Fluorinated naphthalene
  - (2) Halogenated derivatives of naphthalenes, such as:
    - (a) Halogenated homologs of naphthalenes, e. g.:
      - Chlorinated methyl naphthalenes, such as -methyl naphthalene
      - Chlorinated ethyl, propyl, or isopropyl naphthalenes
    - (b) Halogenated amino derivatives of naphthalene, e. g.:
      - Chlorinated naphthylamines
      - Mono-chlor naphthyl amine
    - (c) Halogenated hydronaphthalenes, e. g.:
      - Chlorinated decahydronaphthalene
      - Chlorinated tetrahydronaphthalene
- IV—Phenanthrene and anthracene and related compounds, such as:
- (1) Chlorinated phenanthrene, chlorinated anthracene
  - (2) Halogenated derivatives of phenanthrene and anthracene, such as:
    - (a) Halogenated homologs, e. g.:
      - Chlorinated 1-methyl phenanthrene
      - Chlorinated 3-methyl phenanthrene
      - Chlorinated 9,10 dimethyl phenanthrene
      - Chlorinated propyl and isopropyl derivatives of phenanthrene such as retene
      - Chlorinated dimethyl anthracenes
      - Chlorinated -methyl anthracene
      - Chlorinated propyl and isopropyl derivatives of anthracene
    - (b) Halogenated amino derivatives, e. g.:
      - Chlorinated phenanthrylamines
      - Chlorinated anthramines
    - (c) Halogenated hydrophenanthrenes and Halogenated hydroanthracenes, e. g.:
      - Chlorinated retene oil (contains hydro retene)
- V—Chrysene, picene, and related compounds, including their derivatives, such as homologs, amino derivatives and other substitution products.
- VI—Bridged ring compounds, such as the terpenes and related compounds, and their derivatives, e. g. chlorinated pinene.
- VII—Heterocyclic compounds, such as pyridine, quinoline, pyrrole, thiophene, and derivatives of them, e. g. mono-chlor pyridine.
- VIII—Nitriles derived from any of the above compounds, e. g.:
- Chlorinated:
    - Benzonitrile
    - Tolunitriles
    - Benzyl cyanide
    - Naphthyl cyanide
    - Xenyl cyanide
    - Cyclohexyl cyanide
- IX—Sulphides derived from any of the above compounds, e. g.
- Chlorinated:
    - Diphenyl sulphide
    - Dibenzyl sulphide
    - Dixylyl sulphides
    - Di-naphthyl sulphides
    - Dixenyl sulphides
    - Dicyclohexyl sulphide
- X—Mercaptans derived from any of the above compounds, e. g.
- Chlorinated:
    - Benzyl mercaptan
    - Phenyl benzyl mercaptans
    - Naphthyl mercaptans
    - Phenyl propyl mercaptans
    - Cyclohexyl mercaptan
- XI—Thiocyanates, e. g.
- Chlorinated:
    - Benzyl thiocyanate
    - Phenyl ethyl thiocyanate
    - Phenyl propyl thiocyanate
    - Cyclohexyl thiocyanate
- Halogen-bearing aliphatic compounds**
- I. Hydrocarbons, e. g.
- Chlorinated or fluorinated hydrocarbons which contain from four to ten or more carbon atoms and certain others containing less than four carbon atoms, e. g.
  - 20 Hexachlor ethane
  - Pentachlor ethane
  - Chlor propane
  - Chlor butane
  - Chlor pentane
  - Fluor hexane
  - Fluor octane
  - Fluor decane
  - Tetrachlor ethylene
  - Hexachlor propylene
  - Chlor butylenes
  - Chlor pentenes
  - Chlorinated unsaturated hydrocarbons obtained from products of partial pyrolytic decomposition of high boiling petroleum hydrocarbons.
  - Chlorinated petroleum wax
  - Chlorinated paraffin wax
  - Chlorinated petrolatum
  - Chlorinated aliphatic fractions of mineral oil
- II. Amines, e. g.
- Primary, secondary, and tertiary, e. g.
  - Fluorinated tri-butyl amines
  - Fluorinated tri-amyl amines
  - Fluorinated hexyl amines
- III. Nitriles, e. g.
- 40 Chlorinated or fluorinated
    - Ethyl cyanide
    - Butyl cyanide
    - Octyl cyanide
    - Lauryl nitrile
    - Stearyl nitrile
- 45 The halogen bearing compounds which may thus be advantageously employed in combination with the sulphur compounds of the type above identified may also desirably contain oxygen and such halogen and oxygen bearing organic compounds may be classified as follows:
- Halogen and oxygen-bearing organic ring compounds**
- Oxygen-bearing derivatives of:
- A. "Carbon ring" type compounds
- (1) of the aromatic, or allied type, including oxygen-bearing derivatives of benzene, naphthalene, anthracene, etc., also compounds of the bridged ring type, such as the terpenes, and related compounds.
  - (2) of the class including the cycloparaffins, cyclo-olefines, etc. Examples of this class are oxygen-bearing derivatives of the following:
    - (a) Hydrogenation products of benzene (e. g. cyclohexane, cyclohexene, cyclohexadiene), such as hydrogenated phenol, notably
      - Cyclohexanol
      - Di-hydro phenol
      - Tetra-hydro phenol
    - (b) Hydrogenation products of naphthalene (e. g. decahydronaphthalene, tetrahydronaphthalene, etc.), such as the hydrogenated naphthols.
    - (c) Naphthenes, such as naphthenic acid, etc.
    - (3) of mixed type such as derivatives of indene, hydrindene, hydranthracene, etc.
- B. "Heterocyclic" type compounds
- (1) of the aromatic or allied type including derivatives of pyridine, quinoline, etc.
  - (2) other types such as furane and its derivatives and derivatives of thiophene, pyrrole, etc.

